

Patented Nov. 7, 1922.

1,434,549

## UNITED STATES PATENT OFFICE.

WARREN K. LEWIS, OF NEWTON, AND HAROLD C. WEBER, OF MILTON, MASSACHUSETTS, ASSIGNORS TO LEWIS, GREEN, McADAM & KNOWLAND, OF BOSTON, MASSACHUSETTS, A COPARTNERSHIP CONSISTING OF WARREN K. LEWIS, WILLIAM GREEN, WILLIAM McADAM, AND RICHARD G. KNOWLAND.

### PROCESS OF FLASH-PROOFING FABRICS.

No Drawing.

Application filed October 16, 1919. Serial No. 331,105.

To all whom it may concern:

Be it known that we, WARREN K. LEWIS and HAROLD C. WEBER, citizens of the United States, residing, respectively, at 5 Newton, in the county of Middlesex and State of Massachusetts, and at Milton, in the county of Norfolk and State of Massachusetts, have invented a new and useful Improvement in Processes of Flash-Proofing Fabrics, of which the following is specification.

This invention relates to processes of reducing the inflammability of fabrics made of vegetable materials such as cotton, jute or 15 flax and is particularly concerned with cotton fabrics which have a nap surface, such as flannelette. One objection to the use of fabrics of this character is the fact that a spark or flame striking the surface of the 20 goods, even for a very brief instant, is liable to set fire to the nap, and the fire so started flashes quickly over the surface of the cloth. Thus there is great danger that fire catching in garments made of material of this 25 character will result in burning the wearer very seriously, even though the fire originated in a manner which would be entirely harmless if the garment were made of a different material. In order to overcome 30 this difficulty attempts have been made heretofore to treat fabrics of this character in a manner designed to render them permanently less inflammable. Processes of this 35 character are frequently termed in the trade "flash-proofing processes" and they will be so designated hereinafter.

The present invention aims to devise a process of flash-proofing fabrics which can be economically practised on a commercial 40 scale and which will give superior results.

According to the present process the flannelette or other fabric to be flash-proofed is first immersed in an aqueous solution of a salt of a metal (other than the alkaline 45 earths) whose phosphate is insoluble. Preferably we use aluminium sulphate. Any desired strength of solution can be used, say, for instance, about 1 per cent. After the fabric has become thoroughly wet with the 50 solution it is removed from this bath and the surplus solution is squeezed out of it by running it through a suitable wringer or mangle. The cloth is next immersed in an

aqueous solution of some soluble phosphate, preferably a sodium phosphate. This solution may be of any suitable strength, say, 1 to 2 per cent. The cloth is then wrung out of the second solution, is washed, and dried. We believe that this process is essentially a process of dyeing with colorless dye. That 60 is, a mordant in the commonly accepted sense of the term is a compound with an affinity for textile fibres on the one hand and for certain specific dye stuffs on the other. The fibre is treated first with a mordant, 65 combination ensuing. The combination of fibre and mordant is then treated with a dye stuff, the dye stuff which otherwise would not combine with the fibre, now combining with the mordant fixed to the fibre, producing a permanent combination. In the same way aluminium sulphate, while not ordinarily considered a mordant for cotton because its affinity for cotton is so much less than its affinity for the animal fibres, wool and silk, does, nevertheless, combine with cotton; when so combined it will then combine with phosphate ion, thereby fixing the phosphate radical to the cotton in exactly the way a mordant fixes a dye to the fibre and securing 70 thereby a result not otherwise obtainable. In other words, the reactions that take place in this process are of the same nature as those that characterize any dyeing process using a mordant. 75

That the result is not due solely to the precipitation of an insoluble compound within the voids of the fibre itself, is proven by the fact that barium sulphate, calcium phosphate and similar insoluble compounds 80 thus precipitated on the fibre are not permanently affixed; they are readily dusted out, whereas the aluminium phosphate is held with great tenacity.

In the process above described the aluminium phosphate is the material that actually 85 does the flash-proofing, but this material is incorporated with the cloth in such a way that it remains permanently in the goods. We have found it impossible to obtain this 90 result simply by mechanically padding or loading the fabric with aluminium phosphate. It is evident, therefore, that something more than a mechanical union between the aluminium phosphate and the fabric 95 is produced by this process.

While we have hereinbefore named the materials that we prefer to use in practising this process, it is obvious that other materials than those specifically mentioned can be used. Inasmuch as it ordinarily is undesirable to have the flash-proofing process affect the color of the goods, the salt in the first bath should be one that will form a colorless combination with phosphate ion. 5  
10 The other material used should be a salt of one of the phosphoric acids. We have also found that the order in which the cloth is treated in the two baths can be reversed. We consider it preferable, however, to treat 15 the cloth finally with the salt of one of the phosphoric acids. We regard it as essential to this process that the cloth be treated successively with two solutions, one of which acts as a mordant, and the active elements 20 in both solutions being capable of reacting with each other to form in the goods an insoluble salt of one of the phosphoric acids.

What is claimed as new is:

1. The process of flash-proofing fabrics which consists in immersing the fabric successively in two solutions, one of aluminium sulphate and the other of sodium phosphate. 25
2. The process of flash-proofing fabrics which consists in immersing the cloth in a solution of aluminium sulphate, squeezing the surplus solution out of the cloth, next immersing the cloth in a solution of sodium phosphate, and finally washing and drying the cloth. 30
3. The process of flash-proofing fabrics which consists in treating the fabric successively with two solutions, one of said solutions containing a soluble aluminum salt, and the other containing a soluble phosphate. 35

In testimony whereof we have signed our names to this specification.

WARREN K. LEWIS.  
HAROLD C. WEBER.